

July 31, 1928.

1,679,197

J. M. AARONS

SETTING STRUCTURE FOR LUMBER KILNS AND THE LIKE

Filed Feb. 16, 1924



Fig. -1



Fig. -2

Jacob M. Aarons  
By Brockitt, Hyde & Milburn

Attorneys

## UNITED STATES PATENT OFFICE.

JACOB M. AARONS, OF CLEVELAND HEIGHTS, OHIO.

## SETTING STRUCTURE FOR LUMBER KILNS AND THE LIKE.

Application filed February 16, 1924. Serial No. 693,282.

This invention relates to setting structures for lumber kilns and the like.

Heretofore, setting structures for kilns and the like have been made with a heat insulating coating on the outside of the setting, with the result that the inner usually porous surface of the setting was subjected to the injurious action of the intense heat and abundant moisture within the kiln compartments, and the outside heat insulating coating was subjected to the deteriorating effects of the elements and climatic changes.

The object of the present invention, therefore, is to provide an improved setting structure for lumber kilns and the like which successfully overcomes the above and other disadvantages of setting structures now in use by forming the structure with a heat insulating coating on the inner surface of the setting. As a result, the life and effectiveness of the structure are materially prolonged.

Further objects of the invention are in part obvious and in part will appear more in detail hereinafter.

In the drawing, which represents one suitable embodiment of my invention, Fig. 1 is a cross sectional view of a two-compartment lumber kiln; and Fig. 2 is a fragmentary perspective view thereof.

In the present embodiment of the invention, the settings of the kiln are of brick work, the kiln comprising side walls 1, a rear wall 2, a front wall 3, and a centrally disposed, longitudinally extending partition 4 dividing the kiln into two compartments 5. The front wall 3 is provided with two doors 6, providing access to each of the compartments.

In order to seal the compartments against the escape of heat, the inner porous surfaces of the side and end settings are each provided with a heat insulating coating. In the present embodiment, this coating comprises a primer coat 7 in liquid form, which is brushed onto or otherwise suitably applied to the brick work to seal the pores thereof, and a second or finishing coat 8 in plastic form, which is applied to the primer coat by a trowel or the like.

A primer coat which has been found particularly satisfactory for this purpose is

made of pine oil and the asphalt material known as uintaite or gilsonite, while a satisfactory finishing coat is made up of asbestos fibres, gilsonite and pine oil. While the heat insulating coating so formed may be of any suitable thickness, a thickness of one-eighth of an inch has been found to be satisfactory.

Lumber kilns and the like are often constructed with a plurality of compartments, and as all of the compartments may not be in use at the same time, it is desirable that each compartment be sealed, so that the heat in any one compartment cannot escape into other and perhaps then idle compartments. My improved setting structure should, therefore, be used for the kiln partitions, both surfaces of each partition setting being provided with a heat insulating coating above referred to. While a setting structure with only one surface of the setting provided with such a coating will prevent the passage of heat therethrough, a setting structure in which both surfaces of the setting are provided with a heat insulated coating is desirable, for the reason that neither surface of the porous setting is subjected to the injurious action of the intense heat and abundant moisture within the kiln compartments or to climatic changes when some compartments are idle.

It will thus be seen that I have provided a setting structure for lumber kilns and the like in which the several kiln compartments are effectively sealed against the escape of heat, and in which the inner porous surface of the setting is not subjected to the injurious action of the intense heat and abundant moisture within the kiln compartments, and the heat insulating coating is not subjected to the deteriorating action of the elements and climatic changes.

Other advantages of the invention will be apparent to those skilled in the art to which it relates.

What I claim is:

1. A setting structure for lumber kilns wherein considerable heat and moisture are encountered, comprising a setting of porous material and a heat insulating and moisture proof coating applied to the inner surface thereof, said coating comprising a primer coat of gilsonite and pine oil and a finishing

coat of asbestos fibres, gilsonite, and pine oil.

2. A setting structure for lumber kilns wherein considerable heat and moisture are encountered, comprising a setting of porous

5 material and a heat insulating and moisture proof coating applied to the inner surface thereof, said coating comprising a primer

coat applied in liquid form made up of gilsonite and pine oil and a finishing coat applied in plastic form made up of asbestos <sup>10</sup> fibres, gilsonite and pine oil.

In testimony whereof I hereby affix my signature.

JACOB M. AARONS.